

## UNITED STATES PATENT OFFICE

2,159,964

## MAGNESIUM ALLOY

Arthur Burkhardt, Berlin-Lichterfelde, and Richard Knabe, Berlin-Zehlendorf, Germany, assignors to Georg Von Giesche's Erben, Breslau, Germany, a corporation of Germany

No Drawing. Application July 2, 1938, Serial No. 217,254. In Germany August 10, 1937

2 Claims. (Cl. 75—168)

Our invention relates to magnesium alloys.

It is an object of our invention to provide a magnesium alloy which possesses high resistance to corrosion and good mechanical properties, and can be used, for instance, in vehicle and aircraft structures.

With the object of our invention in view, we make our alloy as follows:

|            | Percent   |
|------------|-----------|
| 10 Bismuth | 2 to 6    |
| Cadmium    | 0.5 to 3  |
| Aluminium  | 1 to 5    |
| Zinc       | 1 to 3.5  |
| Magnesium  | Remainder |

15 The remainder or base may be pure, or commercially pure, magnesium, or it may consist substantially of magnesium, i. e., a low percentage of a component usually employed in magnesium alloys for improving certain properties, may be added to the remainder or base.

20 Magnesium alloys as known at the present time are not quite satisfactory. They either possess high resistance to corrosion or good mechanical properties, but there is no magnesium alloy in which both features are combined.

25 Thus, a magnesium alloy which is resistant to corrosion, has poor tensile strength, of the order of 30 kilogrammes per square millimetre. Conversely, if the tensile strength is increased to, say, about 38 kg. per sq. mm., by heat treatment or by suitable additions to the alloy, the alloy is not resistant enough to corrosion. Moreover, such high-tensile alloys are sensitive to internal stress and suffer from intergranular corrosion. Addition of manganese improves their corrosion resistance but deteriorates their mechanical properties, particularly their toughness, while it does not cure the two weaknesses aforesaid, since the segregation of the strength-increasing components along the grain boundaries is not suppressed, or the hardening component is not dissolved homogeneously but appears as a second phase.

30 Our novel alloy, on the other hand, is equal to the best magnesium alloys known in corrosion resistance, but far superior in mechanical properties.

According to our invention, corrosion resistance is not produced by adding known corrosion-preventing metals but by suitable selection of the components and by determination of the concentration of saturated mixed crystals, preventing the formation of a second phase of the hardening component.

35 The single-phase alloys thus produced are distinguished by the absence of the heterogeneous inclusions acting as local elements in other magnesium alloys of high strength. At the same

time, strength is considerably improved by the formation of the mixed crystals. If the strength of the alloy is increased by hardening and tempering, segregation does not occur along the grain boundaries but is distributed uniformly so that the heat-treated alloy is free from sensitivity to internal stress, and from intercrystalline corrosion.

The preferred percentages of the component in our novel alloy are as follows.

|                |           |
|----------------|-----------|
| Bismuth        | 4 to 5    |
| Cadmium, about | 2         |
| Aluminium      | 2 to 4    |
| Zinc, about    | 3         |
| Magnesium      | Remainder |

15 The remainder is substantially all magnesium, i. e. it may contain an addition which is usually made in magnesium alloys for improving certain properties, for example, 0.1 to 1% of the following metals; manganese for improving corrosion resistance; calcium for improving castability; silicon or a metal of the iron group, i. e., iron, nickel, or cobalt, for increasing the strength of the alloy at high temperature, and its yield point.

The following table gives examples of several magnesium alloys according to our invention, the remainder being substantially magnesium in all cases.

| Alloy No. | Bismuth, percent | Cadmium, percent | Aluminium, percent | Zinc, percent | 30 |
|-----------|------------------|------------------|--------------------|---------------|----|
| 1         | 5                | 2                | 3.5                | 3             |    |
| 2         | 4                | 2                | 4                  | 3             |    |
| 3         | 4                | 2                | 5                  | 3             |    |
| 4         | 5                | 3                | 2                  | 2             | 35 |
| 5         | 2                | 3                | 5                  | 3             |    |
| 6         | 6                | 0.5              | 5                  | 3.5           |    |
| 7         | 6                | 3                | 1                  | 2             |    |
| 8         | 4                | 3                | 5                  | 1             |    |

40 It was found that alloy No. 1, in extruded condition, has a tensile strength of 30 to 45 kg. per sq. mm., and an elongation of 12 to 5%, and that its resistance to corrosion, as tested in the salt spray apparatus with 3% common salt solution, is practically equal to that of electron, AZ 855, 45 with 8% aluminium, 0.5% zinc, 0.1 to 0.3% manganese, remainder magnesium.

We claim:

1. A magnesium alloy containing 2 to 6% bismuth, 0.5 to 3% cadmium, 1 to 5% aluminium, 1 to 3.5% zinc, the remainder substantially all magnesium.

2. A magnesium alloy containing 4 to 5% bismuth, about 2% cadmium, 2 to 4% aluminium, about 3% zinc, the remainder substantially all magnesium.

ARTHUR BURKHARDT.  
RICHARD KNABE.